

May 19, 1936.

G. A. RICHTER

2,041,666

## CYCLIC PROCESS OF TREATING ALKALINE PULPS

Original Filed Dec. 4, 1925



## UNITED STATES PATENT OFFICE

2,041,666

CYCLIC PROCESS OF TREATING  
ALKALINE PULPSGeorge A. Richter, Berlin, N. H., assignor to  
Brown Company, Berlin, N. H., a corporation  
of MaineApplication December 4, 1925, Serial No. 73,193  
Renewed September 26, 1930

23 Claims. (Cl. 92—9)

This invention has relation to the production of a high alpha cellulose fiber, that is, a fiber containing a high percentage of alpha or resistant cellulose and having certain optimum characteristics, from a pulp derived from the digestion of wood chips in an alkaline liquor, and more particularly in a kraft or sulphate liquor.

Wood pulp, as produced by an alkaline digestion, such as kraft, is especially characterized by its quality of high strength, which renders such pulp industrially valuable for use in the manufacture of strong papers, e. g., wrapping and bag papers. Such pulp, however, is inferior in respect of tear resistance and folding endurance, 15 to the high grade manila, or rope pulps, so called, which find extensive use in cable insulation papers and in the manufacture of bags, and various other products, where the characteristics of high tear resistance and folding endurance, as well as 20 strength, are of prime importance.

Moreover, such alkaline pulps are exceedingly difficult to bleach. While it is possible to bleach kraft pulp with an excessive amount of bleach, say, about 50% of 35% lime bleach ( $CaOCl_2$ ) 25 based on the weight of dry pulp, the strength of the resultant bleached pulp is materially lowered and its alpha cellulose content undergoes a material decrease by conversion or degradation into oxycelluloses, so that the commercial value of 30 such pulp is lowered. This difficulty in bleaching may be directly traced to the high percentage of non-alpha cellulose constituents in the form of lignous matter, less-resistant celluloses and other coloring substances present in a pulp derived from the alkaline digestion of wood chips. 35 Nor is it possible to remove to any great extent these non-alpha cellulose constituents, by treating such alkaline digested pulps at elevated temperature with a relatively dilute alkaline solution, as is described in application Serial No. 72,522 filed December 1, 1925, by Milton O. Schur and myself, as being successful in connection 40 with the treatment of sulphite pulp.

In working with or producing various pulps, I 45 have discovered that if an alkaline digested pulp, such as kraft, is treated with a relatively concentrated, cold alkaline liquor, e. g., a solution of caustic soda, I am enabled to produce a fiber having a very high tear resistance and very good 50 folding endurance, and which may thus be employed as a manila fiber substitute. The change in the characteristics of the pulp, which has been effected by the alkaline treatment, doubtless arises from the fact that the treatment purifies 55 or frees the pulp from the pentosans, less-resist-

ant celluloses, lignous and other non-alpha cellulose constituents contained therein, without perceptibly injuring its alpha cellulose content, thereby converting it into a pulp which is especially high in alpha or resistant cellulose content.

Even after such alkaline treatment, however, the pulp does not yield to a bleaching treatment very readily, and requires an excessive amount of bleach to be converted into a white pulp. The 10 use of such excessive bleach materially affects the fiber strength of the pulp and the alpha cellulose content thereof, as previously stated. I have further discovered, however, that the necessity for the use of excessive bleach may be avoided 15 by treating a thoroughly cooked raw pulp prior to the alkaline treatment, with a small quantity of oxidizing or chlorinating agent, such as a chlorine solution. This preliminary treatment is in no sense a bleaching operation, for the color 20 of the pulp is not materially changed. The chlorine, it appears, reacts with and forms soluble compounds with lignous and other coloring substances contained in the pulp, or conditions the pulp by rendering such substances more susceptible 25 to the dissolving or removing reaction exercised thereupon by the alkaline liquor in the subsequent treatment. After the alkaline treatment, the pulp may be bleached with a moderate amount of bleach into a white pulp of high alpha 30 cellulose content suitable for use in the manufacture of high grade writing papers, or for other purposes where a pulp of high alpha cellulose content is required.

The kraft pulp employed in the present invention may be produced, as ordinarily, by the digestion of wood chips (spruce, for example) in a digester, under the requisite time, temperature, and pressure conditions in accordance with modern practice, in the usual kraft or sulphate liquor 40 containing sodium sulphide, sodium hydroxide, and a relatively slight or adventitious amount of sodium sulphate. Spruce, hemlock, pine, or any other raw cellulosic material suitable for the production of kraft pulp may be utilized. After the 45 necessary period of digestion, the digester contents are blown and the kraft pulp is washed and separated from its accompanying black spent digesting liquor.

The washed pulp is then preferably screened 50 to remove shives, specks, and other contaminating matter, and, if desired, is partially bleached as hereinbefore described. It is then thickened to the consistency desired for admixture with a liquor containing the alkaline compounds em- 55

ployed for purification. The thickened pulp is then intimately mixed with a solution containing caustic soda or other equivalent alkaline compounds and is treated therewith, say at room 5 temperature (30° C.), for a sufficient period of time to permit the alkaline solution to react with and remove the non-alpha cellulose constituents of the pulp. In carrying out the treatment or purification only with caustic soda, too high a 10 concentration of caustic soda must be avoided, since otherwise the fiber of the pulp will become mercerized (such mercerization tending to lower the strength of the pulp), and subsequent beating merely macerates or shreds the pulp, without effecting its hydration, so that paper made therefrom is extremely weak. On the other hand, if too low a concentration of caustic soda is employed, a sufficient purification or reaction upon the impurities contained in the pulp, by the caustic 15 soda solution, will not take place and the resulting pulp will not be sufficiently high in alpha cellulose. In other words, the concentration of caustic soda employed in the alkaline treatment is maintained between two limits, namely, between a maximum concentration at which mercerization takes place and a minimum concentration at which a sufficient purification of the pulp is not effected. These limits will vary somewhat, depending upon the temperature or treatment 20 employed and the differences in character of the initial raw stock. After the purification, the pulp containing a high percentage of alpha cellulose is washed free from its treating liquor and may be employed as a manila fiber substitute, as previously indicated. If desired, the treated or purified fiber which still possesses the tan or brownish color of the raw kraft pulp may be bleached at a stock consistency of about 10% to 16% with about 5% to 10% of 35% lime bleach 25 (CaOCl<sub>2</sub>), based on the dry weight of fiber, without materially affecting its strength, tear resistance, folding endurance, and alpha cellulose content, to a color which closely approximates or simulates the light yellow tinge of high-grade 30 manila fiber.

In certain cases, however, it is desirable to produce from raw alkaline digested pulps a pure white product which is characterized by its high alpha cellulose content, and which is suitable for 35 use as a "new rag" substitute in the manufacture of high grade writing papers as well as in the preparation of cellulose derivatives, such as the cellulose esters and ethers, and in the manufacture of such products as artificial silk. If the 40 raw pulp is treated with a chlorinating or oxidizing agent, such as a chlorine solution or bleach liquor, for a relatively short period of time prior to treatment with an alkaline solution, and is then treated with a solution of a suitable alkaline 45 compound, the pulp is sufficiently freed or purified from its non-alpha cellulose constituents to permit the purified pulp to be bleached with a moderate amount of bleach without perceptible injury to its strength or decrease in its alpha cellulose content. If a pulp of exceptionally high whiteness is desired, such pulp may, if desired, be superbleached in a chlorine or other suitable solution.

In certain cases, it may be of advantage to 50 place a portion or all of the caustic soda used in the alkaline treatment by a suitable amount of other alkaline compound, such as sodium sulphide, which exerts a similar purifying or refining action on the raw pulp. For instance, substantially equivalent results to those outlined

may be obtained by treating a raw alkaline digested pulp with a solution of sodium sulphide of somewhat higher concentration than that of a solution of caustic soda. When the caustic soda is replaced by a substantial proportion of 5 sodium sulphide or in entirety thereby, mercerization of the fiber of the pulp is generally precluded, since sodium sulphide does not readily cause a mercerization of cellulose fiber.

While I have indicated that the alkaline purifying or refining treatment is ordinarily carried out at room temperature, it may be stated that lower than room temperature (say, 0° C. to 25° C.) may be employed in such treatment. Likewise, higher temperatures (for example, 25° C. to 75° C.) and a correspondingly suitable concentration of alkaline compound may be employed in such treatment. Thus, in effecting the purification of kraft pulp with a white liquor utilized for digesting wood chips in a kraft mill, a very good product was obtained at a treating temperature of 75° C. In this connection, I have observed that a more highly concentrated alkaline solution should be associated with a higher treating temperature in order to avoid causing 25 a mercerization of the fiber and injury to the papermaking characteristics of the pulp. For instance, in order to treat raw pulp successfully at 30° C. with the usual white liquor of a kraft mill without mercerizing the fiber, such liquor 30 must be diluted with about 50% water, whereas the treatment, as indicated, may be carried out without the dilution of the liquor at 75° C. This observation is in line with the generally known principle that mercerization may be more readily 35 effected at low temperatures. In actual practice, the lower the temperature employed in the purification treatment, the greater the care which must be exercised to avoid such a high concentration of alkali as to cause mercerization. 40

The present invention may be practised advantageously in connection with a plant wherein raw alkaline digested pulp, such as either a kraft or soda pulp, is produced. The soda pulp herein referred to is preferably a long-fibered pulp approximating the strength of kraft, i. e., a pulp produced from the digestion of raw cellulosic material, such as spruce or pine. Such kraft or soda pulp may be employed as the raw material for the production of a high alpha cellulose fiber 50 possessing the properties of very high tear resistance, and folding endurance, and stability.

A more complete understanding of the present invention may be obtained from the following description, when considered in conjunction with the accompanying diagrammatic and conventional drawing, which represents what may be termed a flow sheet showing the course or flow of the various materials employed in the process. The invention will now be described as applied in connection with the kraft process of fiber liberation, but it will be obvious that it may be employed in connection with the soda process.

Referring to the drawing, at 1, I have indicated a digester in which raw cellulosic material in the form of wood chips may be placed and digested in an alkaline liquor for the production of an alkaline pulp suitable for use as a raw material in the preparation of the finished high alpha cellulose fiber, herein desired. After the chips 70 have been cooked in an alkaline cooking liquor comprising a solution of caustic soda and sodium sulphide, under the necessary time, temperature, and pressure conditions in accordance with modern practice, to effect a liberation of fiber, the

digester contents are blown into a suitable blow pit 2, wherein the pulp is separated from its spent black digesting liquor, which is delivered from the blow pit into a black liquor storage tank 3.

5 The alkaline raw pulp, together with its associated spent black liquor, is withdrawn from the blow pit by a pump 4 and delivered therefrom into a counter-current washer, consisting of a series of pulp washers indicated conventionally at 10 5. The washer is preferably of the counter-current type illustrated and described in U. S. Letters Patent No. 1,421,664, to Brown Martinson et al., although, if desired, the ordinary rotary vacuum type of washer may be employed. In the 15 washer of the patent referred to, the pulp is carried continuously through tanks in one direction and the washing liquor is carried successively through such tanks in the opposite direction. The clean wash water is passed from a pipe 7 to the 20 pulp delivered at the last washer of the series from which the washed pulp is delivered. The washed pulp may be delivered from the washer by a conduit 9 through the usual screens indicated conventionally at 10, from which it is delivered 25 to a mixing tank 11, wherein it is intimately mixed with a solution of alkaline compounds necessary for the purifying treatment. The spent black liquor which is associated with the pulp is passed from the first pulp washer of the series by a conduit 13 into the black liquor storage tank 3.

A part of the black liquor from the tank 3 may be withdrawn by a pump 130 and by-passed through a pipe 14 into the digester 1, wherein it is reemployed, together with a freshly prepared 35 cooking liquor, for the digestion of another batch of wood chips. The remaining portion is delivered through a pipe 15 into an evaporator 16 wherein a part of the aqueous content of the liquor is removed prior to the incineration of its 40 combustible content and the recovery of its inorganic mineral content.

The concentrated liquor from the evaporator 16 is delivered through a pipe 17 into a recovery retort 20 and smelted under reducing conditions, 45 thereby producing a smelt consisting essentially of sodium sulphide and sodium carbonate. For making up losses in the digesting cycle, sodium and sulphur in the form of salt cake may be introduced into the concentrated spent liquor 50 from a storage tank 18 through a pipe 19 prior to the incineration or smelting of the black liquor. Or, if desired, the loss in sulphur and sodium constituent in the cycle may be made up 55 by adding free sulphur and caustic soda to the concentrated spent liquor prior to introduction to the furnace.

The hot molten effluent from the furnace is delivered into the water contained in the dissolving tank 21 from which the resultant heated 60 smelt liquor may then be passed through the pipe 22 into a causticizing tank 23, wherein it may be treated, while being agitated, with sufficient lime to causticize or convert its carbonate content to caustic soda. The heated liquor is then filtered 65 as usual, as by passage through a rotary filter 24, for the removal of the calcium carbonate precipitate and foreign matter. The heated, filtered white liquor is delivered from the filter 24 by a pump 25 through a pipe 26 into the white liquor 70 storage tank 27 from which it is next delivered by a pump 28 through a pipe 29 into the digester 1, wherein it is utilized for the liberation of fiber together with the reemployed portion of black liquor. A portion of the white liquor in the 75 tank 27 may, however, be used for admixture with

the raw stock in the mixing tank to effect the purification of such stock, as will presently be described.

Reverting now to the alkaline stock which has been delivered into the tank 11, as shown, provision is made for uniformly or intimately mixing such stock with a solution containing alkaline compounds, e. g., caustic soda, for its purification. To this end, the stock in the tank is treated, while being agitated, with a solution containing 10 alkaline purifying compounds fed thereinto in controlled and regulated amount by way of a feeding device 30 from a pipe 36. The stock, together with the treating solution uniformly admixed therewith, is withdrawn from the mixing tank 15 by a pump 31 and passed into a thickener 32, wherein it is concentrated or thickened to the consistency desired in the purifying treatment, say about 6% to 16%. The white water extracted 20 from the stock in the thickening operation is passed from the thickener 32 through a pipe 33 into a storage tank 34 from which it is withdrawn by a pump 35 and passed through the pipe 63 into the mixing tank 11, wherein it is reused for admixture with other raw alkaline stock to be purified. Thus the white water which is removed from the thickening operation and recirculated to the mixing tank merely serves as a vehicle or carrier for effecting a thorough mixture and distribution 25 of caustic soda throughout the stock. Such thorough mixing can only be obtained with a dilute stock containing excess carrier which is reemployed in the cycle. The stock is allowed to undergo the purification treatment at relatively low 30 temperatures, which may range from lower than room temperatures up to 75° C., as previously indicated. When a solution of only caustic soda is employed, the maximum concentration thereof is below that at which the mercerization of the alpha cellulose content occurs, and the minimum above 35 that at which a sufficient purification is not effected. For optimum results in respect to alpha cellulose content in the finished product, at a temperature of about 30° C. the minimum and maximum concentrations in a stock suspension 40 of about 5% or 6% are, respectively, about 100% and 150% caustic soda based on the weight of dry fiber. The alkalinity of the caustic soda solution is thus about 5% to 7½% caustic soda strength. 45 At this temperature the stock usually requires about one hour to undergo purification, or, in other words, to complete its passage through both treating tanks. Of course, the time of treatment or temperature may be varied, as desired, depending upon the characteristics of the raw stock. 50

The purified stock, together with the tremendous excess of unused caustic soda contained in the liquor, is passed through a counter-current washer 38 of a type similar to that previously described, wherein it is washed free from its alkaline constituents. The washed and purified stock is withdrawn at one end of the washer, through 55 the conduit 39.

The spent liquor which is withdrawn at the other end of the washer contains a large amount of free caustic. Thus, if a caustic solution contains 100% caustic soda based on the dry weight of stock at the time when it enters the reaction tank 34, approximately 90% of this caustic soda 60 remains unconsumed or unconverted after the purifying treatment has been effected, so that, obviously, the larger portion of the liquor from the washer may be reutilized for the purification of other raw alkaline stock. As shown, such spent 65

liquor is passed from the washer through the conduit 40 into an intermediate storage tank 41, from which it is withdrawn by a pump 42 and delivered through a conduit 36 into the feeding device 30 which serves to regulate the supply of purifying solution going to the mixing tank 11. In order to avoid an accumulation of organic matter which has been removed from the raw alkaline stock, however, provision is made to divert a certain small portion of spent liquor obtained from the counter-current washer 38, either to the evaporated liquor prior to its incineration, or for use together with alkaline liquor for the liberation of fiber from wood chips in the production of the raw alkaline pulp. In the drawing, I have shown a pump 45 which delivers a portion of such spent liquor from the washer 38 through a pipe 46 to the evaporator 16, but this portion may be bypassed into the digester 1, if desired. This volume diverted for evaporation or use in the digester may approximate 10% of the total spent liquor.

For the replenishment of losses occasioned in the supply of alkaline compounds used in the purifying treatment, provision is made for continuously removing a certain small portion of strong, hot white liquor from the storage tank 27 to make up such losses. To this end, I have shown a pump 50 which withdraws a portion of such hot white liquor from the tank 27 and forces it through a pipe 51 and a cooler 52, thence through a pipe 53 into the intermediate storage tank 41, from which it is supplied to the feeding device 30 for admixture with raw alkaline stock. Such an arrangement allows the process to be carried out in a very economical manner. Thus, when the purifying treatment is carried out in connection with a raw alkaline pulp derived from the digestion of wood chips by the kraft process, as outlined, the treating or purifying liquor for such alkaline pulp will contain a certain portion of sodium sulphide as well as sodium hydroxide. Such a liquor has been found to serve the purpose of converting kraft stock to a high alpha cellulose containing fiber possessing the properties of very high tear resistance and folding endurance. However, when the process is carried out in a plant wherein chips are digested in a solution of sodium hydroxide, obviously, then, the purifying treatment is carried out with caustic soda alone as the purifying reagent.

However, in a kraft pulp plant favored by a cheap electrical supply so that sodium hydroxide may be manufactured economically, that is, where local and economic conditions permit, a modification of the hereinbefore described procedure may be advantageous. The raw materials for carrying out the process in such case may consist of sodium hydroxide and sulphur, rather than salt cake, and the sodium constituent for the entire process beginning with raw chips and terminating in a high alpha cellulose product may be introduced into the cycle by adding caustic soda as the make-up chemical to the intermediate storage tank 41 from the caustic soda tank 55 (indicated in dotted outline); and the make-up sulphur in the kraft mill may be introduced into the furnace from a tank 53 (indicated in dotted outline), together with the concentrated spent liquor. Of course, the amount of sodium constituent diverted to the kraft mill from the purifying treatment will be sufficient to make up sodium losses occasioned therein. With such an arrangement, even though the purification treatment of the alkaline pulp is practised in connection with the

kraft process, no sodium sulphide will be present in the purifying liquor. Under conditions where the purifying treatment is carried out with sodium hydroxide alone, the resulting purified fiber is more easily bleachable, especially when it has been pretreated with an oxidizing agent.

In certain other cases it may be of advantage to change the described procedure to one wherein all the spent liquor obtained from the washer 38 is employed, instead of the filtered hot white liquor, for the cooking of wood chips in the digester 1. In other words, the procedure may be one wherein all of the liquor from the white liquor storage tank 27 is employed as a purifying liquor, and all of the liquor from the purifying treatment is utilized in the digester 1 for the liberation of raw fiber from chips. Inasmuch as only a small proportion of the total alkaline content in the white liquor from the counter-current washer 38 has actually been converted to inert or inactive constituent in the purifying treatment, the strong liquor from the washer 38 has substantially the same concentration of sodium sulphide and caustic soda under certain conditions hereinbefore stated, as the white liquor in the storage tank 27. This being the case, it may be used in the digester 1 for cooking fresh chips, rather than recirculated to the mixing tank 11, as shown in the drawing. With such an arrangement, the hot white liquor from the storage tank 27 may be passed through a cooler prior to its passage through the control feeding device 30 and into the mixing tank 11, if low temperature is employed in the purification treatment. On the other hand, if a full strength white liquor, with which a treating temperature of 75° C. should be associated, is used in the purification treatment, it is, of course, employed without cooling.

Among the advantages flowing from the practice of the hereinbefore described procedure, is that I am able to produce, with a high yield, from raw alkaline digested pulp, a fiber having a high alpha cellulose content and possessing a very high tear resistance and folding endurance. The physical characteristics of the purified fiber are very similar to the manila fiber such as is used in making a high grade paper for cable insulation.

I present herewith a table showing certain characteristics of an ordinary raw kraft stock prior to and after the alkaline treatment, the various figures representing the averages obtained by making tests on different batches of similarly treated pulp;

|                          | Kraft pulp | Purified pulp            | 55 |
|--------------------------|------------|--------------------------|----|
| Mullen strength (beaten) | 155-160    | 120-142.                 |    |
| Tear                     | 220-245    | 350-400.                 |    |
| Alpha cellulose, %       | 88-89      | 93-96.                   |    |
| Pentosans, %             | 7-10       | 3-5.                     |    |
| Folding endurance        | 1800-2400  | 3000-4000<br>double fold | 60 |
| Yield of process, %      |            | 92-95.                   |    |

From the foregoing table, it will be seen that the tear resistance of the original pulp has undergone a considerable increase at the expense of its so-called Mullen strength and that the alpha cellulose of the original pulp has been increased and its pentosan correspondingly decreased.

By utilizing a thoroughly cooked unbleached kraft pulp as a raw material, I have further found that a white product suitable for use as a "new rag" substitute in the manufacture of writing papers may be produced by subjecting the pulp to a preliminary oxidizing or chlorinating treat-

70  
75

ment prior to the alkaline treatment or purification, as hereinbefore indicated. Such pretreatment conditions the pulp for the alkaline treatment and allows the pulp to be bleached after the 5 alkaline treatment with a moderate amount of bleach and without perceptible injury to its strength or decrease in its alpha cellulose content. The pretreatment is, however, apt to lower the yield of final product somewhat. In such 10 case, the pulp is pretreated approximately at a stock density of about 5%, preferably with a solution containing 1% to 2% chlorine or 2% to 6% of 35% lime bleach ( $\text{CaOCl}_2$ ) based on the dry weight of fiber. The oxidizing agent reacts with 15 the difficultly removable non-alpha cellulose constituents contained in the pulp, forming soluble reaction products, or products more easily removable by the subsequent alkaline treatment. The pretreated stock is then purified in a solution of 20 alkaline compounds, as hereinbefore described.

Since the pretreatment and subsequent alkaline purifying treatment have removed from the raw alkaline digested pulp a substantial amount of non-alpha cellulose constituents, the purified 25 pulp can be bleached with materially less hypochlorite or bleach than is required without such treatments, to produce a pure white product; and this bleaching operation may be effected without material injury to the strength of the purified 30 pulp, or reduction of its alpha cellulose content. Ordinarily, a bleaching treatment at a stock consistency of about 10% to 16% with about 5% to 10% of 35% lime bleach ( $\text{CaOCl}_2$ ) based on the dry weight of pulp, is sufficient to bring the pulp 35 up to a whiteness equivalent to or approximating that of ordinary bleached sulphite pulp.

The stock thus bleached may be improved in color by a superbleaching operation, which may be carried out at a stock consistency of from 4% 40 to 6%, with about .2% to 5% chlorine, based on the weight of dry fiber.

Owing to its properties resulting from the purifying treatment which it has received, the white high alpha cellulose fiber may be employed 45 not only as a substitute for "new rag" fiber in the manufacture of high grade bond and ledger papers, but also in the manufacture of the cellulose esters and the cellulose ethers, and for other purposes where a substantially pure cellulose 50 fiber is required.

Thus, by the practice of this invention, I am enabled to increase the tear resistance and folding endurance of the raw alkaline digested pulp at the expense of its Mullen strength, and also 55 to purify it into a product which is especially high in alpha cellulose. This is highly desirable, since the tear resistance and its accompanying quality of folding endurance are of extreme importance in high grade papers, whereas the Mullen or bursting strength is usually of secondary 60 importance. This may be better understood from the fact that it is relatively easy to increase the Mullen or bursting strength of a paper sheet by suitable beating and sizing. The beating and 65 sizing operations, however, do not affect the tear test so appreciably, so that it is a distinct advantage to increase the tear test even at the expense of the strength of the pulp, inasmuch as it is possible to increase the strength by special 70 treatment.

Moreover, paper manufactured from an unbleached purified pulp as herein produced, because of its softness and absorbency, is admirably adapted for many uses to which a harsh or 75 ratty paper could not be put. For example, such

paper may be employed for the production of artificial reed fiber, such as serves in the manufacture of baby carriages, furniture, etc. Such a paper should have a high tear resistance, should be soft and yet firm, and should have sufficient 5 porosity to permit its ready impregnation with glue, varnish, or other waterproofing reagents. Such paper can be produced from the product resulting from the herein described process.

Before concluding, it may be stated that, while 10 I have specified certain concentrations of stock and treating compounds in order to more fully and adequately describe my invention, these concentrations may vary, depending upon plant equipment and other conditions. That is to say, 15 the plant equipment with which the present invention was practiced permitted the treatment of an alkaline digested stock at a concentration of about 5% to 6%, most efficiently and successfully. On the other hand, a stock concentration of 10% 20 or greater may be treated under other plant conditions. In such cases, the percentage of caustic soda or other alkaline compounds utilized in the purification may be correspondingly adjusted. The determining factors in carrying out 25 the purifying treatment or reaction are the concentration of the alkaline compounds in the liquor and the temperature at which the liquor is used. Of course, if sodium sulphide or some other reagent, which is less drastic or effective in its 30 reaction than caustic soda, is used, the percentage of such reagent may be increased in order to produce a product substantially equivalent to that obtained by the use of caustic soda.

The change in the characteristics of the raw 35 alkaline digested pulp is effected with a relatively high yield of finished high alpha cellulose product, the yield ranging from 93% to 95%, based on the weight of dry, raw pulp.

At the risk of repetition, it may be stated that 40 the drawing is wholly diagrammatic and conventional, no attempt having been made to show the true size relationship between the various instrumentalities, or their proper location. For the sake of clarity in the drawing, certain details of 45 construction have been omitted, but it will of course be understood that fittings, pipes, pumps, devices for controlling temperature conditions, or any other apparatus necessary for maintaining the flow of the various materials or for 50 maintaining certain conditions, will be supplied wherever necessary.

I do not herein claim the subject matter of my application, Serial No. 28,339, filed May 6, 1925, which discloses the recovery of alkaline compounds of spent liquor employed in the treatment of cellulose pulp together with the alkaline compounds of spent kraft liquor; nor do I herein 55 claim the subject matter of the hereinbefore identified application, which discloses an alkaline 60 digestion of sulphite pulp at elevated temperature.

Having thus described this invention and a method of practicing the same, it should be obvious to those skilled in the art that various 65 changes and modifications in procedure might be resorted to without departing from its spirit or scope as defined by the appended claims.

What I claim is:

1. A process which comprises treating with a 70 liquor containing fresh alkaline sodium compounds, pulp derived from the digestion of wood chips in a digesting liquor containing sodium compounds, reutilizing one portion of alkaline liquor resulting from such treatment in the alkaline 75

treatment of other pulp, and smelting and recovering the sodium compounds from the other portion of such liquor, together with the sodium compounds of said spent digesting liquor, in the 5 form of alkaline sodium compounds.

2. A process which comprises treating with a liquor containing fresh alkaline sodium compounds, pulp derived from the digestion of wood chips in a digesting liquor containing sodium compounds, reutilizing one portion of alkaline liquor resulting from such treatment in the alkaline treatment of other pulp, smelting and recovering the sodium compounds from the other portion of such liquor, together with the sodium compounds of said spent digesting liquor, and adding sufficient alkaline sodium compounds to said first mentioned portion to carry out the alkaline treatment of other pulp.

3. A process which comprises treating with a liquor containing fresh alkaline sodium compounds, pulp derived from the digestion of wood chips in a digesting liquor containing sodium compounds, reutilizing one portion of alkaline liquor resulting from such treatment in the alkaline treatment of other pulp, smelting and recovering the sodium compounds from the other portion of such liquor, together with the sodium compounds of said spent digesting liquor, in the form of alkaline sodium compounds, and adding sufficient alkaline sodium compounds from the recovered alkaline sodium compounds to said first mentioned portion to carry out the alkaline treatment of other pulp.

4. A process which comprises treating with a liquor containing fresh alkaline sodium compounds, raw pulp derived from the digestion of wood chips in a digesting liquor containing alkaline sodium compounds, utilizing alkaline liquor resulting from such treatment as digesting liquor for the liberation of other raw pulp from wood chips, smelting and recovering the sodium compounds from said digesting liquor in the form of alkaline sodium compounds, and utilizing the recovered compounds in an alkaline liquor for the treatment of other raw pulp.

5. In purifying unbleached pulp prepared from wood by an alkaline process, the sequence of operations which comprises partially bleaching the pulp, treating the partially bleached pulp with a solution of caustic alkali, the pulp and solution being brought together in such amounts and concentrations as to give a resulting suspension having an alkalinity equivalent to that of a caustic soda solution of at least about 5% strength but below mercerizing strength, continuing the treatment for the desired period of time at a temperature less than the boiling point of water, separating caustic alkali solution from the so-treated pulp and washing the latter, subjecting the treated and washed pulp in aqueous suspension to a second stage of bleaching treatment, and washing the resulting finally bleached pulp.

6. A process which comprises subjecting unbleached alkaline wood pulp to a preliminary bleaching treatment with a fraction of the total bleaching agent required, admixing the partially bleached pulp with a solution of caustic alkali of such concentration and in such proportion that the resulting mixture has an alkalinity equivalent to a solution of caustic soda of at least about 5% strength but below mercerizing strength, maintaining the mixture at a temperature below 212° F. for the desired period of time, separating caustic alkali solution from said mixture and washing the pulp, subjecting the washed pulp to

a secondary bleaching treatment with the rest of the bleaching agent required, and washing the resulting pulp.

7. A process which comprises subjecting unbleached sulphate pulp obtained from coniferous wood to a preliminary bleaching treatment with a fraction of the total bleaching agent required, thickening the bleached pulp, admixing with the thickened pulp a solution of caustic alkali of such concentration and in such proportion that the resulting mixture has an alkalinity equivalent to a solution of caustic soda of at least about 5% strength but below mercerizing strength, maintaining the mixture below 212° F. for the desired period of time, separating caustic alkali solution from the mixture and washing the pulp, subjecting the washed pulp to a secondary bleaching treatment with the rest of the bleaching agent required, and washing the resulting pulp.

8. A process which comprises subjecting unbleached sulphate pulp obtained from coniferous wood to a preliminary bleaching treatment with a fraction of the total bleaching agent required, thickening the partially bleached pulp, admixing therewith caustic soda solution in such amount and concentration as to bring the resulting mixture to a consistency of about 6% of dry pulp substance with an alkalinity of the resulting solution equivalent to about 6.5% of caustic soda, maintaining the mixture at less than the boiling point of water for about one hour with agitation, separating caustic soda solution from the mixture and washing the pulp, subjecting the washed pulp to a secondary bleaching treatment with the rest of the bleaching agent required, and washing the resulting bleached pulp.

9. A method for the treatment of cellulosic materials which comprises reducing the same to the condition of pulp by cooking with an aqueous solution containing an alkaline sulphide, removing resulting solution from the remaining pulp, and treating the latter with an aqueous alkaline solution of a reactive compound of sulphur.

10. A method for the treatment of cellulosic materials which comprises reducing the same to the condition of pulp by effecting incomplete cooking with an aqueous solution containing an alkaline sulphide, removing the resulting solution from the pulp and treating the latter with a reactive compound of sulphur in alkaline solution.

11. In purifying unbleached chemical wood pulp, the sequence of operations which comprises partially bleaching the pulp, washing the partially bleached pulp, treating the partially bleached and washed pulp with a solution of caustic alkali, the pulp and solution being brought together in such amounts and concentrations as to give a resulting suspension having an alkalinity equivalent to that of a caustic soda solution of from about 5% to about 12% strength and a pulp concentration of from about 5% to about 10%, continuing the treatment for from about 10 minutes to about 6 hours, separating caustic alkali solution from the so-treated pulp and washing the latter, subjecting the treated and washed pulp to a second stage of bleaching treatment, and washing the resulting finally bleached pulp.

12. A method for the treatment of cellulosic materials which comprises reducing the same to the condition of pulp by cooking with an aqueous solution containing an alkaline sulphide, removing resulting solution from the remaining pulp, and treating the latter with an aqueous alkaline solution of sodium sulphide.

13. A method for the treatment of cellulosic materials which comprises reducing the same to the condition of pulp by effecting incomplete cooking with an aqueous solution containing an alkaline sulphide, removing the resulting solution from the pulp, and treating the latter with sodium sulphide in alkaline solution. 5
14. A method for the treatment of cellulosic materials which comprises reducing the same to 10 the condition of pulp by cooking with an aqueous solution containing an alkaline sulphide, removing resulting solution from the remaining pulp, treating the pulp with a bleaching agent, and then treating the pulp with an aqueous alkaline solution of a reactive compound of sulphur. 15
15. A method for the treatment of cellulosic materials which comprises reducing the same to the condition of pulp by cooking with an aqueous solution containing an alkaline sulphide, removing resulting solution from the remaining pulp, treating the pulp with a bleaching agent in amount insufficient to bring the pulp to substantial whiteness, then treating the pulp with an aqueous alkaline solution of a reactive compound 20 of sulphur, and again treating the pulp with sufficient bleaching agent to bring it to substantial whiteness. 25
16. A method for the treatment of cellulosic materials which comprises reducing the same to 30 the condition of pulp by cooking with an aqueous solution containing an alkaline sulphide, removing the resulting solution from the remaining pulp, treating the pulp with a bleaching agent, and then treating the pulp with an aqueous alkaline solution of sodium sulphide. 35
17. A method for the treatment of cellulosic materials which comprises reducing the same to the condition of pulp by cooking with an aqueous solution containing an alkaline sulphide, removing resulting solution from the remaining pulp, treating the pulp with a bleaching agent in amount insufficient to bring the pulp to substantial whiteness, then treating the pulp with an aqueous alkaline solution of sodium sulphide, and again treating the pulp with sufficient bleaching agent to bring it to substantial whiteness. 40
18. A method for the treatment of cellulosic materials which comprises reducing the same to the condition of pulp by cooking with an alkaline liquor containing caustic soda, removing result- 45
- ing liquor from the remaining pulp, and treating the latter with an aqueous alkaline solution of a reactive compound of sulphur. 5
19. A method for the treatment of cellulosic materials which comprises reducing the same to 10 the condition of pulp by cooking with an alkaline liquor containing caustic soda, removing resulting liquor from the remaining pulp, and treating the latter with an aqueous alkaline solution of sodium sulphide. 15
20. A method for the treatment of cellulosic materials which comprises reducing the same to 20 the condition of pulp by cooking with an alkaline liquor containing caustic soda, removing resulting liquor from the remaining pulp, treating the pulp with a bleaching agent, and then treating the pulp with an aqueous alkaline solution of a reactive compound of sulphur. 25
21. A method for the treatment of cellulosic materials which comprises reducing the same to 30 the condition of pulp by cooking with an alkaline liquor containing caustic soda, removing resulting liquor from the remaining pulp, treating the pulp with a bleaching agent in amount insufficient to bleach the pulp to substantial whiteness, then treating the pulp with an aqueous alkaline solution of a reactive compound of sulphur, and again treating the pulp with sufficient bleaching agent to bleach it to substantial whiteness. 35
22. A method for the treatment of cellulosic materials which comprises reducing the same to 40 the condition of pulp by cooking with an alkaline liquor containing caustic soda, removing resulting liquor from the remaining pulp, treating the pulp with a bleaching agent, and then treating the pulp with an aqueous alkaline solution of sodium sulphide. 45
23. A method for the treatment of cellulosic materials which comprises reducing the same to the condition of pulp by cooking with an alkaline liquor containing caustic soda, removing resulting liquor from the remaining pulp, treating the pulp with a bleaching agent in amount insufficient to bleach the pulp to substantial whiteness, then treating the pulp with an aqueous alkaline solution of sodium sulphide, and again treating the pulp with sufficient bleaching agent to bring it to substantial whiteness. 50

GEORGE A. RICHTER. 50